

## 1

3,169,288

COATINGS FOR PATTERNS EMPLOYED IN  
CAVITYLESS CASTING PROCESS

John L. Dewey, Pleasant Hill, Calif., assignor to The Dow Chemical Company, Midland, Mich., a corporation of Delaware  
No Drawing. Filed Dec. 15, 1961, Ser. No. 157,245  
2 Claims. (Cl. 22—195)

This invention relates to an improved pattern for use in the preparation of foundry castings. More particularly, it relates to such patterns for use in the fabrication of castings by the so-called cavityless technique.

It has been proposed heretofore to prepare metal castings by embedding in a mold body a pattern formed from a material that is substantially completely volatile or combustible upon contact with the molten metal of a casting charge, providing the mold body with a pour opening and a vent opening, each communicating with the embedded pattern, and then pouring the casting charge into the pour opening. Contact between the entering molten metal and the pattern is effective to cause the rapid volatilization or decomposition of the latter so that it is completely destroyed, leaving behind a cavity in the mold body to be filled by the casting charge.

The above-described method of producing castings possess certain manifest advantages not to be found in the conventional molding practice which, for the casting of any but the most simple forms, requires rigorous attention to coring and the providing of proper parting lines in the mold. In the described method a casting of any degree of complexity can be produced without regard to these factors. Parting lines need not be provided for, inasmuch as the casting may readily be formed in one piece. Elements of the structure of the casting conventionally provided by coring are readily produced by proper design of the destructive or fugitive pattern.

It is obvious that the fugitive pattern should possess as small a mass per unit volume as is possible, so that, for a given material of its construction, the heat required for its destruction be minimal and the volume of the gaseous products of its volatilization be as small as possible. The heat is, of course, supplied by the casting charge and, if too great a quantity of heat be abstracted therefrom, localized solidification may occur which may result in the production of inferior castings.

Foamed, thermoplastic, resinous materials, such as polystyrene foam, are ideally suited to the production of these fugitive patterns. They possess the necessary strength to remain dimensionally stable during the embedment of the pattern in the mold body. The actual weight of material in the pattern is small. This, coupled with the volatility of the resinous foam, makes for rapid and complete burn-out of the pattern upon the pouring of the casting charge.

One major difficulty, however, attends the use of foamed thermoplastic resins. Advantageously, and usually, the pattern is fabricated from a solid block of such foamed resin, or component parts thereof are cut or carved from the foamed resin and are then assembled into the desired shape. Cutting through the foamed resin necessarily gives a surface that is rough and pitted, inasmuch as a multiplicity of open cells constitutes the said surface.

## 2

This surface pattern is transferred to the mold body in contact therewith and is thus duplicated on the surface of the casting.

It has been suggested that the surface of such a pattern be smoothed by the application of a hot iron. This expedient has only limited value, however, since it is virtually impossible to maintain the dimensions of the pattern by this technique. Furthermore, in the case of a pattern of complex shape, the difficulty of following the contours thereof with the smoothing iron are such that the method cannot successfully be employed.

It is therefore the principal object of the invention to provide a destructible pattern of a foamed, resinous thermoplastic material, the use of which in cavityless casting results in the production of castings having desirably smooth surfaces.

It is an additional object of the invention to provide a means of imparting smoothness to the surface of a destructible pattern of the type described without sacrifice of the dimensional accuracy thereof.

Other and additional objects of the invention will be evident from the description to follow.

According to the present invention, destructible patterns of foamed, thermoplastic resinous materials are given a smooth surface by the application of a coating material that is effective to fill up the open pores or pits of the surface of the pattern. As a result, that portion of the mold body which is in contact with the surface of the embedded destructive pattern does not assume the rough surface characteristics of the resinous foam but rather the smooth surface characteristics of the applied coating. The casting produced in the mold so prepared is accordingly possessed of a smooth surface and, as a consequence, requires the minimum of surface finishing. Maintenance of dimensional accuracy in the casting is readily realized.

Preferably, the pattern coating material should be substantially non-fugitive. That is, it should not be destructive on contact with the casting charge to give rise to any substantial volume of gaseous products of thermal decomposition or of volatilization, the rapid exit of which products from the mold body through the pour opening may result in spattering of the molten metal being poured. Furthermore, excessive gas formation at the mold body-metal interface is undesirable. Such gas formation, coupled with the cooling effect of volatilization of a fugitive coating material and heat absorption by the mold body, can cause surface defects in the casting by preventing intimate contact of the metal with the mold surface while localized solidification of the metal may be taking place.

The pattern coating material must be essentially non-adherent to the face of the mold body under the conditions of high temperature prevailing during casting. A related requirement is that the coating should not retain its form when subjected to this high temperature. If these conditions are not met, the volatilization of the pattern will leave the inside wall of the mold body faced with the coating material having a rough surface derived from the rough surface of the fugitive pattern.

Finally, the coating material should not give rise to slag during casting. Slag formation is known to result in the production of inferior castings.

All of these aforementioned desirable attributes for a coating for fugitive patterns employed in cavityless casting are possessed by the coatings of the present invention.

The coating compositions of the present invention comprise admixtures of at least one pulverulent refractory material, a binding agent for the aforesaid refractory material and an aqueous dispersing medium therefor. Optionally, and advantageously, the compositions may also contain a dispersing agent.

The refractory materials, of course, are the major constituents of the coating obtained from the coating compositions. They perform the principal function of filling the imperfections or voids in the pattern surface with a material that will not melt or lead to slag formation during the casting operation. The binding agent serves to maintain the coating in a coherent form so that it will not be lost from the surface of the pattern during the handling of the latter during its embedment in the mold body.

The dispersing agent is included in the composition to aid in obtaining uniform admixture of the other components in the aqueous dispersing medium, and to aid in maintaining the desired consistency of the composition. This consistency can be adjusted so that the product takes the form of a relatively fluid composition suitable for spray or brush application to the pattern, or it may be paste-like and adapted to application with a spatula, trowel or the like.

After application of the coating composition thereto, the pattern may be allowed to stand at ambient temperature until substantial dehydration of the composition has taken place. Preferably, however, it may be exposed to an elevated temperature to hasten the dehydration, which temperature necessarily is below that at which the pattern would be adversely affected.

The dried coating is smooth, hard and adherent to the pattern surface. It is of sufficient strength to withstand the stresses imposed upon it during embedment of the pattern in the mold body. In foundry practice, for example, the coating remains intact during the sand ramming operation and the sand at the sand-coating interface is readily provided with the smooth surface desirable for metal casting.

When the coating material is subjected to the elevated temperature of the molten casting charge, the coating loses its cohesiveness. Because of the loss of its cohesiveness, the coating assumes a pulverulent form rather than retaining the rough surface reflective of that of the now destroyed pattern with which it was in contact. Inasmuch as its actual volume is small, its presence exerts little if any measurable effect on the dimensions of the finished casting. The major portion of this pulverulent material is swept out of the cavity through the vent openings by the gaseous products of the thermal decomposition of the fugitive pattern resulting from the pouring of the casting charge.

A wide variety of refractory materials may be employed in the preparation of the coating compositions of the present invention. Fire clay, bentonite, silica, alumina and fine zircon sand are representative. Advantageously, bentonite will constitute a portion of the refractory component, being used in conjunction with a second refractory material. The use of bentonite aids measurably in dispersing the other refractory material in the aqueous medium. Additionally, its presence in the composition lends considerable stability thereto. In general, the bentonite will be employed in an amount equal to from about 8.0 percent to about 10.0 percent of the total weight of refractory material.

The binding agent may be chosen from the wide range of materials that are known to be useful in the preparation of molds and cores of foundry sand compositions, such as cereal, flour, asphaltic emulsions, thermoplastic resinous composition dispersions and the like. A preferred type of binding agent is represented by polyelec-

trolytes such as water soluble or dispersible salts of polyacrylic acid or polymethacrylic acid, polyacrylamide, polyaminoalkylacrylates, polyvinylpyridine and the like. A large number of these polyelectrolytes are known to the art and are employed to improve the handling characteristics of wet sand-clay mixtures in the preparation of foundry sand molds. When an agent of this type is employed in the practice of the present invention, it imparts to the coating composition a desirable smoothness and consistency in addition to performing its function as a binding material in the dried coating.

The preparation of the coating compositions of the present invention, as well as the mode of their use, is described in the following non-limiting examples, where-in all parts and percentages are given on a weight basis.

#### Example 1

To 1000 parts of water there were added, with rapid stirring, 50 parts of bentonite followed by 1.5 parts of anhydrous sodium pyrophosphate. To the resultant dispersion there were slowly added 1.2 parts of polyacrylamide with continued stirring, after which 50 parts of pulverulent fire clay were thoroughly admixed with the thick slurry obtained to give a stiff pasty mass suitable for application to a pattern surface by troweling.

#### Example 2

Following the procedure of Example 1, a relatively fluid mixture was prepared from 1000 parts of water, 35 parts of bentonite, 40 parts of pulverulent fire clay, 1.5 parts of sodium pyrophosphate and 1.1 parts of polyacrylamide. To this mixture there were added, slowly and with rapid mixing, an additional 100 parts of bentonite. An extremely thick, smooth paste resulted.

#### Example 3

Following the procedure of Example 1 a coating composition was prepared from 1000 parts of water, 40 parts of bentonite, 140 parts of pulverulent fire clay, 1.5 parts of sodium pyrophosphate and 1 part of polyacrylamide. The resultant mixture was sufficiently fluid for brush application to the surfaces of a fugitive pattern.

#### Example 4

The coating composition of Example 2 was smoothly applied to the rough surfaces of a block of foamed polystyrene with a spatula. The composition was allowed to dry for 4 hours at 120° F. A hard, smooth, adherent coating resulted.

The thus coated block was embedded, according to known procedure, in a foundry sand mold body. A pour opening and a vent were provided in the mold body. A charge of molten steel at 3000° F. was added through the pour opening. The resultant casting was found to possess a smooth surface comparable to that of the coated pattern.

In contrast thereto, the casting obtained when an uncoated block of foamed polystyrene was employed as the fugitive pattern possessed the rough, pitted surface characteristic of the pattern.

#### Example 5

A block of foamed polystyrene was coated, by brush application, with the coating composition of Example 3. The coating obtained after drying of the composition was smooth and hard and the casting resulting from the use of the coated block as a fugitive pattern was free from surface roughness and pitting.

What is claimed is:

1. In a process for casting of metals which comprises making a pattern mold with destructive patterns of foamed, thermoplastic resinous materials with surfaces corresponding to the desired casting embedded in said mold, and the pouring of molten metal into said mold

whereby the foam pattern is destroyed and a metal casting is obtained, the improvement which comprises depositing on the surface of the pattern a coating of an aqueous suspension of an admixture of at least one pulverulent inorganic refractory material and a binding agent therefor and causing the removal of water from the deposited wet coating whereby to provide the pattern with a smooth, dry, adherent, cementitious coating.

2. The process of claim 1 wherein bentonite constitutes at least about 8 percent by weight of the total weight of the pulverulent refractory material.

5

2,120,526  
2,623,809  
2,830,343  
2,836,867  
3,070,991

767,114

## References Cited in the file of this patent

## UNITED STATES PATENTS

Owen ----- June 14, 1938  
Myers ----- Dec. 30, 1952  
Shroyer ----- Apr. 15, 1958  
Bean ----- June 3, 1958  
Holbrook et al. ----- Jan. 1, 1963

## FOREIGN PATENTS

Great Britain ----- Jan. 30, 1957